

## UNITED STATES PATENT OFFICE

2,565,938

LUBRICANT METAL-ROLLING  
COMPOSITION

Robert C. Williams, Columbus, Ohio, assignor to  
The Ironsides Company, Columbus, Ohio, a corporation of Ohio

No Drawing. Application May 11, 1949,  
Serial No. 92,729

6 Claims. (Cl. 252—57)

1

The present invention relates generally to lubricating materials or compositions, and more particularly to an improved lubricant composition for use with metals undergoing various types of forming operations, such as gauge reduction between the rolls of a cold-rolling mill.

In the past, the generally accepted material used as a lubricant for metals undergoing rolling operations was palm oil, or a mixture of palm oil with other materials or ingredients, such as certain liquid hydrocarbon vehicles or solvents. The primary objections to the use of palm oil as a lubricating material stem from the fact that this material is generally an imported product whose availability and cost are subject to extreme fluctuation, and whose physical properties and chemical composition are subject to relatively wide variation. A major disadvantage in the use of palm oil as a lubricant material for metal rolling operations is caused by a relatively wide variation in the free fatty acid content of different shipments or batches of palm oil as received at the import market. As is well known, the free fatty acid content of imported palm oil may vary generally between approximately ten per cent and upwards of thirty-five per cent, depending upon the time interval between production and use and the temperatures to which the same has been subjected during production, storage and use; it being understood that the free fatty acid content of palm oils generally increases due to a breaking down of the natural vegetable fats and fatty acid compositions during sustained periods of storage, particularly where such storage is effected in relatively high temperature climates.

It will be manifest that a relatively high free fatty acid content within a lubricant rolling material is particularly disadvantageous for use with metals which are intended to undergo plating or tinning operations after rolling, due to the fact that such metals are generally subjected to cleaning or washing operations with relatively strong alkalies or bases, such as sodium hydroxide, which react with free fatty acids to form soaps or certain saponification products which greatly interfere with the complete cleaning of the metal preparatory to tinning or plating operations.

Furthermore, palm oils have a natural tendency to break down under relatively elevated temperature conditions, such as are encountered during rolling operations, and thereby form or produce an excess of free fatty acids which, in the event that the palm oil is used with an emulsify-

2

ing agent, oftentimes causes an imbalance of the emulsifying agent, resulting in an unstable emulsion.

It is, therefore, the primary objective of the present invention to provide a lubricant composition for use in metal rolling operations which possesses improved operational characteristics over previously accepted palm oil compositions and which may be produced from relatively inexpensive and readily available materials at a fraction of the cost of palm oil or palm oil compositions, and which may be easily compounded and supplied to the user with a predetermined desired percentage of free acids.

It is another object of this invention to provide a lubricant rolling composition whose free acid content may be critically controlled so as to fall within ranges desired for various types of metal-forming operations, and particularly where metals are to undergo subsequent plating or tinning operations.

It is still a further object of this invention to provide a lubricant composition for metal-forming operations which may be supplied to the user with a more or less definite and known acid content without requiring the user to resort to time-consuming and expensive analyses of the lubricant material prior to its use to determine the percentage of acid content therein or to take steps to adjust the acid content prior to the use of the material.

Yet another object of the present invention is to provide a lubricant composition which may be compounded from an inexpensive by-product of a pulp paper-making process, known as tall oil, which has a relatively high and stable free acids content and a solid fat material, such as the better grades of beef or mutton tallow, which are solids at ordinary room temperatures, and which preferably have a free fatty acid content ranging from less than one to five percent and well below the range of acid content of the tall oil, whereby a simple proportional compounding of these two separate ingredients results in end products of buttery consistency having desired and known percentage ranges of free acids commensurate with the requirements of various metal-forming operations.

The present improved lubricant composition comprises an intimate and homogeneous mixture of a normally viscous liquid material (at ordinary room temperatures), known as tall oil, and a normally solid (at ordinary room temperatures) animal or hydrogenated vegetable fat or oil having a free fatty acids content not to exceed 5

percent by weight of the fat or oil and a titre point ranging between 27° C. and 45° C.

Tall oil is a viscous oily liquid at ordinary room temperatures and is obtained as a by-product from the wood of coniferous trees during the process of conversion of the wood fiber into cellulose by the sulphite paper-pulp process. It is a mixture of rosin acids and fatty acids with a small percentage of higher alcohols and generally has a free acids content ranging from 80. to 95 percent by weight of the material.

Preferably, a high grade beef or mutton tallow is used as the principal ingredient of the present lubricant composition, although certain grades of other solid animal fats or oils, such as horse fat or lard, or certain types of hydrogenated vegetable or animal oils which are hydrogenated sufficiently to be solid at ordinary room temperatures, may be employed with substantially equal results. It will be understood, however, that the animal or vegetable fat or oil ingredient should have a relatively low free fatty acids content, preferably ranging from less than one to four percent by weight of the material and not to exceed five percent by weight. Also, the animal or vegetable fat or oil used must be solid at ordinary room temperatures (approximately 20° C. to 25° C.) and preferably has a titre or solidification range of from 27° C. to 45° C.

It has been found that lubricant rolling compositions used in the cold rolling of sheet metal to effect gauge reduction of the metal should preferably have a semi-solid, buttery consistency and a relatively low free acids content, preferably ranging from 6 to 14 percent by weight of the lubricant composition. This limitation upon the percentage of free acids, particularly fatty and rosin acids, is necessitated by the fact that an excessive amount of free fatty or rosin acids in a lubricant rolling composition for sheet metals results in the formation of excessive amounts of soaps or other saponification products when the sheet metal is subjected to washing or cleansing prior to tinning or plating operations with caustic alkalies or bases, such as sodium hydroxide, or alkaline salts, such as sodium phosphates, which washing or cleansing operations are more or less standard practice in preparing sheet metal for tinning operations after rolling. It has further been found that lubricant compositions or materials having a free acids content higher than approximately 15 percent by weight, when used in conjunction with an emulsifying agent for application to the metal as an emulsion, tend to cause instability within the emulsion which results in inefficient lubrication of the metal during forming operations.

Hence, it is the ordinary practice of the metal-forming industry, and particularly rolling mills, to specify that lubricant materials or compositions be supplied which have a free acids content not to exceed 15 percent by weight of the composition, and preferably in two ranges, namely: 6 to 8 percent and 10 to 14 percent, and a semi-solid or buttery consistency in order that the same may be applied to the metal in a number of different ways consistent with the particular type of work being done in an efficient and economical manner.

As a specific example of the production of the present lubricant composition to yield an end product having a free acids content within the range of 6 to 8 percent by weight of the composition, 96 pounds of beef tallow having a titre or solidification point of approximately 37° C. and

a free fatty acids content of 3 percent by weight were blended at approximately 50° C. with 4 pounds of tall oil having a free acids content of 85 percent by weight. The mixture was then allowed to cool to ordinary room temperatures (approximately 25° C.) to provide 100 pounds of a buttery solid lubricant composition having a total acids content of 6.28 percent by weight of the composition. It will be noted that this figure of 6.28 percent is well within the desired lower range of 6 to 8 percent of free acids, and allows for a slight increase in the percentage of free acids, such as might be occasioned by prolonged storage of the material at relatively elevated temperatures prior to use of the material without exceeding the desired upper limit of 8 percent.

As an example of the compounding of the present lubricating composition to provide a total free acids content within the aforementioned desired higher range, viz. 10 to 14 percent, 90 pounds of beef tallow having a titre point of approximately 37° C. and a free fatty acids content of 3 percent by weight were blended with 10 pounds of tall oil having an average free acids content of 85 percent by weight at approximately 50° C. After cooling to room temperatures, the mixture yielded 100 pounds of a homogenous buttery solid composition having a total free acids content of 11.2 percent by weight of the composition.

Thus it will be seen from the foregoing data that by a relatively simple proportional compounding of the two ingredients, preferably beef tallow and tall oil, which have known acid values, the present lubricant composition may be supplied in the desired ranges for total free acids content. It will be understood that should it be desired that the composition have an exact or specific free acids content within the range of 6 to 14 percent, the requirements for such an exact content may be easily satisfied by a simple mathematical determination of the amounts of the separate ingredients required, knowing the acid value thereof, and thereafter by blending the pre-determined amounts together.

It has been found that the present lubricating composition having a free acids content ranging between 6 and 15 percent has given excellent results when used as a lubricant in metal rolling operations where gauge reductions of the order of 65 percent have been effected when operating upon relatively hard metals, such as double A chrome steel. The present lubricant composition is further characterized by its ability to withstand the relatively extreme high pressures encountered during rolling operations without breaking down to yield an undesirably high percentage of free fatty or rosin acids which greatly impede subsequent tinning or plating operations as beforementioned. It has further been noted that the use of the present composition during rolling operations apparently reduces objectionable scale formation upon the metal after initial gauge reduction rolling and during annealing and pickling operations and provides a highly desired bright and lustrous finish upon the metals after the same undergo final finishing or pinch rolling operations.

In use, the present lubricant composition may be applied in its buttery solid form to the sheets of metal or the rolls of the rolling mill prior to or during rolling operations by dripping or spraying the same thereon, by dipping the sheet metal into the composition, or by placing a quan-

tity of the composition within a porous fabric or cloth bag and thereafter permitting the bag to wipe the surface of the sheets or rolls during rolling operations. The present composition may also be applied to the metal or the rolls of a mill in an emulsion form in water, where either mechanical agitation or an emulsifying agent is employed to maintain the material in its emulsified condition. Further, the present lubricating composition may be diluted or cut with a suitable hydrocarbon solvent or liquid vehicle, such as kerosene, and applied in liquid form to the metal prior to or during rolling operations.

In view of the foregoing, it will be noted that the present invention provides an improved and versatile lubricant rolling composition for use with metals undergoing forming operations, such as gauge reduction between the rolls of a rolling mill. The present composition is characterized by its ability to be compounded from relatively low cost and readily available domestic materials which, when combined in definite relative proportions, produce a composition whose properties excel the highest grades of imported palm oils as a lubricant for metal-forming operations. The present lubricant is further characterized by the fact that the same may be supplied with a relatively low, known, and stable free acids content in comparison with the oftentimes high and extremely variable free acids content of imported palm oils or palm oil compositions, thereby enabling the present composition to be used as a lubricating material for metals which are intended for subsequent tinning or plating operations which require that the metal be relatively free from free acids, without resorting to expensive and time-consuming analyses to determine the acid content of the lubricant prior to its use and thereafter taking steps to adjust the acid content of the lubricant to adapt the same for particular uses. Another important advantage to the use of the present composition stems from its physical property of being a buttery or pasty solids material at ordinary room temperatures, thereby enabling the same to be efficiently and economically applied to the metal undergoing forming operations in a variety of ways.

I claim:

1. A lubricant composition for metals undergoing forming operations consisting essentially of a non-flowing mixture of 1 to 17 parts of tall oil having a free acids content of from 80 to 95 percent by weight with 83 to 99 parts of a fat normally solid at ordinary room temperatures

having a free fatty acids content not to exceed 5 percent by weight and a titre point ranging between 27° C. and 45° C., and wherein the total free acids content of said mixture is less than 15 percent by weight thereof.

2. A lubricant rolling composition consisting essentially of a non-flowing mixture of tall oil having a free acids content ranging between 80 and 95 percent by weight and a fat normally solid at ordinary room temperatures having a free acids content ranging between 1 and 5 percent by weight in the following approximate ranges of proportions by weight of the composition:

Tall Oil, 1 to 17 parts

Solid Fat, 83 to 99 parts

the said composition having a total free acids content of 6% to 14% by weight thereof.

3. A lubricant rolling composition of solid non-flowing consistency having a total free acids content of 6% to 14% by weight of the composition and consisting essentially of a homogenous mixture of from 83 to 99 parts by weight of tallow having a free fatty acids content of from 1 to 5 percent by weight and from 1 to 17 parts by weight of tall oil having a total acids content of from 80 to 95 percent by weight.

4. A lubricant rolling material of solid non-flowing consistency having a total free acids content of from 6 to 8 percent by weight of the material and consisting essentially of a mixture of 4 parts by weight of tall oil and 96 parts by weight of a tallow having a free fatty acids content not to exceed 5 percent.

5. The composition set forth in claim 2 emulsified in aqueous solution.

6. The composition set forth in claim 2 diluted with kerosene.

ROBERT C. WILLIAMS.

#### REFERENCES CITED

The following references are of record in the file of this patent:

#### UNITED STATES PATENTS

| Number    | Name     | Date          |
|-----------|----------|---------------|
| 8,176     | Selgrath | June 24, 1851 |
| 1,919,125 | Patch    | July 18, 1933 |
| 2,258,552 | Harris   | Oct. 7, 1941  |
| 2,270,319 | Lieber   | Jan. 20, 1942 |
| 2,326,387 | Nill     | Aug. 10, 1943 |
| 2,377,106 | Reswick  | May 29, 1945  |
| 2,417,283 | Zimmer   | Mar. 11, 1947 |